

# United States Patent [19]

[ 19 ]

[11] 3,905,804

Scott, Jr.

[45] Sept. 16, 1975

- [54] **METHOD OF DECARBURIZATION OF SLAG IN THE ELECTROSLAG REMELTING PROCESS**

[75] Inventor: **William W. Scott, Jr., Parkesburg, Pa.**

[73] Assignee: **Lukens Steel Company, Coatesville, Pa.**

[22] Filed: **June 7, 1973**

[21] Appl. No.: **367,941**

[52] U.S. Cl. .... **75/11**

[51] Int. Cl.<sup>2</sup> .... **C21C 05/54**

[58] **Field of Search** .... **75/10 R, 10 C, 11, 12,  
75/13; 164/52, 252**

**[56] References Cited**

UNITED STATES PATENTS

- |           |         |                |        |
|-----------|---------|----------------|--------|
| 1,645,126 | 10/1927 | Browne.....    | 75/12  |
| 3,650,311 | 3/1972  | Fritsche.....  | 164/52 |
| 3,672,428 | 6/1972  | Tommaney ..... | 164/52 |

## FOREIGN PATENTS OR APPLICATIONS

- 1,150,201 4/1969 United Kingdom..... 164/252

## OTHER PUBLICATIONS

- Metals, 2 (10), March 1967, pp. 44, 45, 46, 47, 46A and 48.  
Duckworth et al., *Electro-slag Refining*, TN 685.5.E4D8, Chapman & Hall Ltd., London, Feb. 2, 1971, (p. 67 relied on).

Mitchell, *Trans. of Metallurgical Society of AIME*, TNLM57, December, 1968, Vol. 242, (pp. 2507-2511 relied on).

British Steelmaker, Sept. 1966, (pp. 48, 49 and 58 relied on).

*Primary Examiner*—L. Dewayne Rutledge  
*Assistant Examiner*—M. J. Andrews  
*Attorney, Agent, or Firm*—Mason, Mason & Albright

[57]

## ABSTRACT

The introduction of an oxidizing agent,  $\text{Fe}_3\text{O}_4$ ,  $\text{FeO}$ ,  $\text{Fe}_2\text{O}_3$ ,  $\text{NiO}$ ,  $\text{MoO}_2$ ,  $\text{CoO}$ ,  $\text{Cu}_2\text{O}$ ,  $\text{Cr}_2\text{O}_3$ ,  $\text{MnO}$ ,  $\text{Mn}_2\text{O}_3$  or  $\text{Mn}_3\text{O}_4$ , or a combination thereof into slag in the bottom of the mold during the beginning of an electro-slag remelting (ESR) process, but after the slag is fully molten and with an a.c. current at about 70 – 90 volts applied through the slag from the ESR consumable electrode in order to reduce the slag's carbon content to less than about 0.02%, the slag having a composition of about 40%  $\text{CaF}_2$ , 30%  $\text{CaO}$ , and 30%  $\text{Al}_2\text{O}_3$ , and having obtained a carbon content of roughly 0.04 – 0.05% upon being melted in a slag furnace having a graphite or carbon brick lining prior to being introduced into the ESR mold, the oxidizing agent being introduced into the slag during the ESR process being about 0.2% of the slag by weight.

**28 Claims, 1 Drawing Figure**





## METHOD OF DECARBURIZATION OF SLAG IN THE ELECTROSLAG REMELTING PROCESS

### BACKGROUND OF THE INVENTION

This invention relates to a method of decarburizing molten slag used in the electroslag remelting process. More specifically it relates to an effective method for removing carbon introduced into the molten slag by reason of being heated to a molten state in a furnace lined with graphite or carbon bricks.

The electroslag remelting process essentially comprises the fusing from a consumable electrode of metal which is to be refined under a blanket of molten slag or flux. The consumable electrode is generally suspended within a water cooled copper or steel mold and molten slag is introduced into the mold and acts as an electrical conductor for electrical current passing between the consumable electrode and baseplate or stool of the mold. The current heats the electrode and droplets of metal fusing off its lower end fall through the slag to the bottom of the mold where a pool of molten metal forms and solidifies upwards from the bottom pool. A refining action takes place in the molten metal as it passes through the molten slag and, as the electrode is progressively consumed, the refined metal builds up from the bottom of the mold to form an ingot. The molten slag floats on the pool of refined metal and remains in contact with the lower end of the consumable electrode. The refining process continues until the electrode is consumed or substantially consumed.

Slags used in electroslag remelting processes have a high dielectric constant in the solid form, but are conductive to some extent in the liquid phase. Also, in the molten state, the slag has a low viscosity and slags utilizing calcium fluoride as one component have a corrosive effect on ordinary refractory. For this reason, a furnace for melting slag prior to its introduction into the mold may be lined with carbon or graphite in brick or monolithic wall form or both. However, it has been found that the graphite or carbon lining, together with the graphite electrodes for melting same, are responsible for introduction of carbon into the molten slag which has presented a problem of removing same. Otherwise, the carbon is transferred to the bottom of the ingot which thus has a higher carbon content than specifications for the steel may call for and, in any event, different from the carbon content at the top of the ingot.

The known method for reducing the carbon level in the molten slag is to blow oxygen into it while in the slag furnace. This method is operable but somewhat unwieldy and it is difficult to estimate when the carbon content has been lowered by the desired amount. Furthermore the carbon or graphite lining is needlessly oxidized by the excess oxygen, causing early failure of the lining.

As an experiment, iron oxide was added to the molten slag in the slag furnace. A highly undesirable foaming action resulted and a crust was formed on the molten slag. It was found, however, by adding the iron oxide very slowly, the carbon content of the slag could be successfully reduced in spite of its foaming action and formation of a crust on the top of the molten slag. The advantages of this method over the introduction of oxygen were that the quantity of carbon removed was more easily gaged and the furnace lining was not detri-

mentally affected. But both methods leave much to be desired in their operational aspects.

### SUMMARY OF THE INVENTION

I have discovered that if the required amount of iron oxide (mill scale,  $Fe_3O_4$ ) is added directly into the mold as soon as practicable after molten slag has been introduced therein and the melting process has commenced, (the slag being in the molten state) the iron oxide can be added at a relatively rapid rate (within 30 seconds to up to five minutes) without causing discernible or harmful foaming or crusting of the molten slag around the consumable electrode. The addition of about 0.2% iron oxide removes about 0.034% carbon from the molten slag. The slag then has a carbon level of about 0.006 - 0.016% which is insufficient to affect adversely the quality of the ingot produced by the process.

Other advantages of the invention will be appreciated from the description and with reference to the accompanying drawing.

### BRIEF DESCRIPTION OF THE DRAWING

The drawing is a schematic view, partly in section which illustrates the preferred mode of carrying out the invention.

### DESCRIPTION OF THE PREFERRED EMBODIMENT

Referring to the drawing, a consumable electrode 10 is suspended by a suspension structure 23 in a water cooled copper or steel mold 11. The mold is supported by a base plate or stool 12 and includes a passageway 18 between the outer shell 14 and the inner mold wall 15. The passageway 18 functions to receive the heat exchange medium 20 for retaining the inner mold wall 15 in an appropriately cooled condition. An inlet 16 and outlet 17 are provided for the cooling medium 20, preferably water. A cap 21 of molten slag or flux receives the lower end of the electrode 10 and, due to heat generated by electric current passing through electrode 10 and cap 21, the lower end of electrode 10 is progressively melted and molten metal drops 22 fall through the cap 21 to form a molten metal pool 24, which, due to the cooling effects of medium 20, solidifies in the form of an ingot 25. The slag blanket or cap 21 is preferably such that it will not liberate deleterious gas either as to quantity or kind during the metal depositing operation and it should not add substantial quantities of undesirable ingredients to or remove substantial quantities of desirable ingredients from the molten metal. Rather it should flux out impurities. The molten slag should, furthermore, be such that it will readily free itself from the molten metal and it has been found that a wide variety of slags or fluxes may be used satisfactorily. A calcium fluoride flux has been found advantageous.

The molten slag which comprises the cap 21 may be passed into mold 11 from a convenient source of supply such as slag furnace 40 by any suitable means as it would occur to one skilled in the art such as the conduit 27 which is preferably water cooled and composed of steel. As shown in the drawing, the conduit 27 enters into the interior of the mold 11 through a snugly fitting opening in stool 12 (which also has cooling passageways designated 19 for receiving cooling medium 20) and also through an opening in a starter plate 28 which is disposed between the stool 12 and the lower ends of

the mold 11. The function of starter plate 28 is to provide a dependable electric conductor under mold 11 to ensure the passage of electrical current when the process is commenced.

The other end of conduit 27 terminates in a funnel portion 29 which is disposed to receive molten slag from spout 41 of slag furnace 40 when it is pivoted around trunnion 42 as indicated in dot-dash lines.

Slag furnace 40 comprises an outer steel shell 44 followed by a layer of compressible fibrous high temperature (2800°F.) insulation 45, fire brick 46, a layer of high alumina refractory bricks 47, an expansion joint 50 comprising powdered alumina, a graphite shell 51 which may be integral and have the shape of a cup or be formed of graphite bricks as shown and finally on the interior a layer of graphite or carbon bricks 52. The roof 54 is composed of a high alumina ram refractory which is tamped in place to form a monolithic roof structure. The roof includes three main openings, an exhaust conduit 55, a feed pipe 56 and a central opening 57 which receives three graphite electrodes 60 which are connected to an appropriate electrical power source not shown. Before slag furnace 40 is pivoted about trunnion 42, the electrodes 60 and roof 56 are raised to the position shown in dot-dash lines.

Dry slag placed within the slag furnace 40 is heated by graphite electrodes 60 and due to its resistance is melted whereby the electrodes become immersed in the slag which is heated to a temperature of 2800° – 2900°F. for tapping.

It has been found that slag furnace 40 gives very few problems and may be used for over 100 heats with bricks 52 replaced every 25 heats more or less. The graphite working lining comprising carbon or graphite bricks 52 together with graphite electrodes 60 introduce, however, more than a desirable amount of carbon into the slag. This carbon, after the slag is introduced into the mold 11, is transferred to the steel forming the ingot 25 so that the carbon content of the ingot is greater in its lower portion than upper portion.

As previously indicated, it is possible to reduce the carbon level in the slag by blowing oxygen into the molten slag bath in slag furnace 40 or by the slow introduction of an oxide such as an iron oxide to the bath which reacts with the carbon to form carbon monoxide and carbon dioxide that is expelled from the molten slag as a gas. Both of these methods have definite drawbacks in that they cause an undue amount of foaming within the slag furnace 40 and also cause a crust to form on top of the slag.

It is my discovery that iron oxide might be directly added into the molten slag in the mold at the appropriate time without causing appreciable or harmful foaming or a crust to form. I am not certain for the reason for this phenomenon but presently am of the opinion that turbulence in the slag cap 21 caused by the passage of electrical current therethrough and the resulting heat causes the gases generated by addition of the oxide to be carried off in such a way that harmful foaming action does not occur.

Iron oxide is added at the top of the mold 11 between the inner mold wall 15 and the sides of the electrode 10 by means of a metering device 61 which meters the desired amount of the oxide into the mold via a pipe 62.

In operation, dry slag material having a composition of about 40%  $\text{CaF}_2$ , 30%  $\text{CaO}$  and 30%  $\text{Al}_2\text{O}_3$ , is added into slag furnace 40 via feed pipe 56 and is melted by

resistance heating between graphite electrodes 60. Additional dry slag is added until the desired amount has been introduced into the slag furnace 40 and the temperature of the slag is brought up to 2800° – 2900°F. Although care is taken to introduce only the amount of slag desired into the slag furnace 40, there is some variability which appears to be inherent in the system and, with the knowledge of such variability, electrode 10 is initially positioned a short but sufficient distance (about 2 inches) from the highest level of slag expected to be introduced within mold 11 from furnace 40 in view of prior experience as to the volumetric parameters of the molten slag charges. The slag furnace 40 is caused by appropriate means (not shown) to tilt about trunnion 42 and thus empty the molten slag into the spout portion 29 of conduit 27 whereupon it enters through said conduit into the bottom of the mold 11. The slag furnace 40 is tilted to over 90° for this purpose in order to ensure that it is emptied insofar as possible of molten slag. When the slag pouring is complete, electrode 10 is promptly lowered at a speed of say 1 inch per 15 – 30 seconds until it contacts the surface of cap 21 whereupon a current flow is immediately registered and cap 21 becomes highly liquid within a relatively short period. However, immediately following contact of electrode 10 with cap 21, there may remain a slight crust at the top of the cap 21 and the addition of any oxide at this time would remain on the crust possibly causing operating problems by arcing for example, although this has not been experienced. After waiting a period of say 5 – 40 minutes when it is known that the crust has disappeared and slag is completely liquid. The oxide can be added and the desired decarburization reactions proceeds. Accordingly, metering device 61 is then activated whereupon the oxide enters the cap 21 via pipe 62 and the space between the inner mold wall 15 and electrode 10.

The amount of iron oxide added depends upon the approximate carbon composition of the slag prior to pouring which, in turn, depends on a number of variables such as the operating technique, the temperature of the slag, the slag chemistry, etc. However, it has been found that two pounds of iron oxide ( $\text{Fe}_3\text{O}_4$ ) per 1,000 pounds of molten slag or, in other words, 0.2% is sufficient to remove about 0.034% carbon from the slag. Inasmuch as the average carbon content of the slag is usually about 0.04 – 0.05%, the carbon level is lowered to a "safe" or tolerable level; that is, less than 0.02% with an aim of about 0.01%, but it is not removed altogether. In the event too much of the oxide is added, the characteristics of the slag may then change from a "reducing" to a "oxidizing" material and oxidizable elements which may be present in the electrode 10 such as aluminum, magnesium, titanium, silicon, manganese, chromium and carbon are taken up by the slag as oxides. Thus, the quantity of oxide to be added is critical and can only be determined for a given facility after the empirical determination of flux carbon content for a number of melts. This, of course, can be accomplished without undue difficulty. However, it is believed that the limits of the oxide addition rate should be kept within a range from 0.1% to 1% in order to remove between about 0.017 to 0.17% carbon in the case of iron oxide ( $\text{Fe}_3\text{O}_4$ ).

It has been determined that the method as disclosed in this invention successfully reduces the carbon in the slag whereby undue carbon content in the lower por-

tion of the ingot 25 is avoided. Whatever minor carbon pick-up affects the bottom of the ingot is eventually eliminated through providing practices.

In the actual reduction to practice of the invention, the interior dimensions of mold 11 within walls 15 are on the order of 20 × 60 inches horizontally and about 115 inches high. Electrode 10 is manufactured so that it can be centered between walls 115 with gaps of about 1½ to 2 inches in width on each side. Furnace 40 has a capacity of about 1½ tons of slag or at least about 2,800 pounds. It takes about 1½ to 2 hours to melt and bring 1,000 pounds of slag to the desired temperature. For 2,800 pounds, the required time is about 3½ – 4 hours. When electrode 10 contacts the top of the slag cap 21, a current flow is immediately registered and an initial voltage of about 90 volts reduces within about a few minutes to about 70 volts with the current being on the order of about 10,000 amps. The current is a single phase 60 cycle a.c. current.

Although  $Fe_3O_4$  is preferable because it is readily available as millscale, other oxides are thermodynamically capable of causing the desired reaction. These include  $Fe_2O_3$ ,  $FeO$ ,  $NiO$ ,  $MoO_2$ ,  $CoO$ ,  $Cu_2O$ ,  $Cr_2O_3$ ,  $MnO$ ,  $Mn_2O_3$  and  $Mn_3O_4$ . A particular oxide may be chosen wherein the metal element involved may be advantageously added for alloying in the lower portion of the ingot, for example, where the lower portion of the electrode contains less than the desired amount of such element. In this connection, it should be understood that the metering device 61 is also utilized in the process involved for the selective addition to the molten slag of materials such as lead, molybdenum, aluminum, copper, chromium, and manganese as and when needed to compensate for deficiencies in the electrode. Moreover, the problem of continually adjusting relative movement between the electrode 10 and mold 11 may be alleviated or, indeed, eliminated by the addition of sufficient steel pellets of desired chemistry of the like from device 62 during the process so that the ingot grows at substantially the same rate that the electrode 10 shortens.

In practice, electrode 10 may be energized prior to or as the slag is charged into the mold 11, or immediately before lowering same. However, preferably, it is energized as slag is charged into the mold. Also, preferably, the slag charging time via funnel portion 29 should not normally exceed four minutes.

For the purpose of the claims, flux is considered to be included in the term "slag." Also, unless otherwise stated, percentages are by weight.

Having thus described my invention, what I claim as new and desire to secure by Letters Patent of the United States is:

1. An electroslag remelting process which comprises: melting of slag in a furnace by means of at least one graphite electrode whereby the carbon content of the molten slag is increased; transferring said molten slag into the bottom of an electroslag remelting mold wherein an ingot of improved homogeneity is formed by the continued melting of a metal consumable electrode the end portion of said electrode being immersed in said molten slag whereby melted metal from said end portion falls through said molten slag and solidifies to form said ingot in said mold while an electrical current passes through said slag between said elec-

trode and said ingot being formed for maintaining said slag in a molten condition; and introducing an oxidizing agent into said molten slag in said mold while said current is passing therethrough, the amount and rate of said introduction of said oxidizing agent being such as to perform the function of removing carbon from said molten slag without causing excessive foaming of said slag.

2. In a method of decarburizing flux having an undesired high carbon content, the flux being used in an electroslag remelting process wherein it is in a molten state in an electroslag refining mold, the lower portion of a consumable metal electrode immersed in the upper portion of the molten flux, the flux being heated by an electrical current flow provided therethrough, melted metal from the electrode passing through said molten flux to the bottom of the mold into a molten metal pool where it solidifies as a more homogeneous metal, the improvement comprising the step of adding iron oxide to said molten flux in said mold while continuing said current flow whereby decarburization of said flux takes place without excessive forming of said flux.

3. A method of accordance with claim 2 wherein the iron oxide added to said flux is about 0.2% of the amount of flux by weight.

4. A method in accordance with claim 3 wherein said iron oxide is mill scale.

5. A method in accordance with claim 3 wherein said iron oxide is introduced into said flux within a time range of 30 seconds to 5 minutes.

6. An electroslag remelting process which comprises the steps of:

heating a charge of slag in a slag furnace to a molten state wherein the slag is exposed to carbon and the carbon content of the slag is increased to an undesired level;

introducing said slag into an electroslag refining mold in its molten state; immersing of the lower end of a consumable metal electrode into said molten slag in said mold and establishing an electric current therethrough which is sufficient to maintain said slag in said mold in a molten state and to melt said electrode immersed therein whereby molten metal is received through said molten slag in a molten metal pool in the bottom of said mold where it solidifies to form a more homogeneous ingot;

immediately with said slag in a molten state after introducing same into said mold, adding an oxidizing agent to said molten slag while continuing said current through said slag and the melting of said electrode whereby the decarburization of said slag takes place without excessive foaming thereof and said slag retains its characteristic as a reducing slag.

7. A process according to claim 6 wherein said oxidizing agent is a substance selected from the group consisting of  $FeO$ ,  $Fe_2O_3$ ,  $Fe_3O_4$ ,  $NiO$ ,  $MoO_2$ ,  $CoO$ ,  $Cu_2O_3$ ,  $MnO$ ,  $Mn_2O_3$  and  $Mn_3O_4$ .

8. A process according to claim 6 wherein said oxidizing agent comprises iron oxide.

9. A process according to claim 8 wherein said iron oxide is mill scale.

10. A process in accordance with claim 6 wherein the amount of oxide added to said slag is about 0.2% of said slag and is introduced in a period of 30 seconds to 5 minutes.

11. An electroslag remelting process which comprises:  
 melting of slag in a furnace which is lined at least in part by carbonaceous material whereby the carbon content of molten slag is increased;  
 transferring said molten slag into the bottom of an electroslag remelting mold wherein an ingot of improved homogeneity is formed by the continued melting of a metal consumable electrode's end portion immersed in said molten slag whereby melted metal from said end portion falls through said molten slag and solidifies to form said ingot in said mold while an electric current passes through said slag between said electrode and said ingot being formed maintaining said slag in a molten condition; and

introducing an oxidizing agent into said molten slag in said mold while said current is passing therethrough, the amount and rate of said introduction of said oxidizing agent being such as to perform the function of removing carbon from said molten slag without causing excessive foaming of said slag.

12. An electroslag remelting process in accordance with claim 11 wherein after said molten slag has been introduced into said mold, said electrode is lowered into contact with said slag and a current flow through said slag is established, the introducing of an oxidizing agent into said slag being thereafter delayed until the slag between said mold and said electrode is in a fully fluid condition.

13. An electroslag remelting process in accordance with claim 12 wherein the period of said delay is about 5 - 40 minutes.

14. An electroslag remelting process in accordance with claim 11 wherein said oxidizing agent is introduced into said slag within a period of less than 5 minutes.

15. An electroslag remelting process in accordance with claim 11 wherein said oxidizing agent is a substance selected from the group consisting of  $FeO$ ,  $Fe_2O_3$ ,  $Fe_3O_4$ ,  $NiO$ ,  $MoO_2$ ,  $CoO$ ,  $Cu_2O$ ,  $Cr_2O_3$ ,  $MnO$ ,  $Mn_2O_3$ , and  $Mn_3O_4$ .

16. An electroslag remelting process in accordance with claim 11 wherein said oxidizing agent consists essentially of iron oxide.

17. An electroslag remelting process in accordance with claim 16 wherein said oxidizing agent consists essentially of mill scale.

18. An electroslag remelting process in accordance with claim 11 wherein said electrical current is an alternating current with a voltage of between about 70 and 90 volts.

19. An electroslag remelting process in accordance with claim 11 wherein about 800 watts of power per pound of slag is being applied to said molten slag when said oxidizing agent is introduced therein.

20. An electroslag remelting process in accordance with claim 19 wherein said oxidizing agent is iron oxide and the amount of said iron oxide added to said molten slag is about 0.1% of the weight of said slag for each 0.02% carbon to be removed from said flux.

21. An electroslag remelting process in accordance with claim 20 wherein sufficient iron oxide is added to lower the carbon content of the molten slag in said mold from the range of about 0.04 to 0.05% carbon to a range of about 0.006 - 0.016%.

22. An electroslag remelting process in accordance with claim 19 wherein the oxidizing agent is mill scale and not more than about 2 pounds of same is introduced to said molten slag for each 1,000 pounds of said slag.

23. An electroslag remelting process in accordance with claim 22 wherein said mill scale is introduced to said molten slag during a period of about one-half minute.

24. In an electroslag remelting process of the type wherein slag is melted in a separate container and sufficient carbon is received by the molten slag in said container so that the carbon content of the molten slag becomes undesirably high, said slag subsequently being introduced into an electroslag refining mold in a molten state, an end portion of a metal consumable electrode being immersed in said molten slag in said mold and an electrical current going through said slag generating heat to fuse metal from the end of said electrode through the molten slag into a molten pool of metal at the bottom thereof where it solidifies to form a metal ingot of improved homogeneity the improvement comprising the step of adding an oxidizing agent into the molten slag in said mold while said current and said molten metal are passing through said molten slag thereby decarburizing said slag without the occurrence of excessive foaming of the molten slag in said mold.

25. In a process according to claim 24 wherein said oxidizing agent comprises iron oxide.

26. In a process according to claim 25 wherein said iron oxide is mill scale.

27. In a process according to claim 24 wherein said electric current is an alternating current of about 60 cycles.

28. In a process according to claim 24 wherein said slag is composed of about 40%  $CaF_2$ , 30%  $CaO$ , and 30%  $Al_2O_3$ .